

## UNITED STATES PATENT OFFICE

2,603,592

## PITCH-LIKE COMPOSITIONS

Harold W. Nelson, Deerfield, Ill., assignor to Great Lakes Carbon Corporation, Morton Grove, Ill., a corporation of Delaware

No Drawing. Application June 15, 1948,  
Serial No. 33,222

14 Claims. (Cl. 196—149)

1

This invention relates to a process for converting raw petroleum coke and the like into valuable pitch-like substances.

Raw petroleum coke and related cokes produced by the pyrolysis of hydrocarbonaceous liquids in non-catalytic processes is a by-product normally useful only as fuels, or after calcination at high temperatures, in the formation of certain carbonaceous articles such as carbon electrodes, anodes and the like. In many localities petroleum coke finds little or no utility and is practically a waste product. This invention provides a method whereby petroleum coke can be converted into substances of wide utility.

According to one specific embodiment the process comprises dissolving a raw, normally non-fusible coke produced by non-catalytic pyrolysis of hydrocarbons, said coke having a volatile content of at least 8%, said volatile content being capable of evolution only upon carbonization, in a suitable high boiling solvent.

The raw cokes useful in this process must have a volatile content of at least 8% and preferably at least 12%. The volatile content may run as high as 30-35%. The term volatile content as used herein refers only to that portion of the coke which is capable of evolution upon carbonization at relatively high temperatures. It does not include water or volatile material, e. g., oil which is entrapped, occluded to, or otherwise mechanically held in the coke.

The raw coke may be produced in the so-called reaction chambers of thermal-non-catalytic cracking plants or may be produced by the coking or carbonization of high boiling residues such as asphalt, crude oil, topped or reduced crude oil, cracked residues, coal tar pitches and the like. Such coke has heretofore been considered to be substantially carbon, but it has been found that it is essentially a high molecular weight, solid hydrocarbon mixture in which the volatile content as contemplated herein is organic and forms a part of the hydrocarbon structure. In contrast to the high melting asphalts which may be produced by the cracking process or upon steam or air reduction of heavy cracked or straight run residues, the raw petroleum coke is non-fusible. Although it can be deformed at temperatures of the order of 500° F. by the application of mechanical pressure, the coke has no melting point and upon simple heating remains undeformed.

I have discovered that coke of this character with a volatile content of 8 to 35% and which is otherwise substantially infusible can be converted into useful products by dissolving or peptizing it in high molecular weight organic solvents. Those

2

solvents are the most useful which are essentially aromatic in character, since they dissolve the coke in the greatest proportions. Among these are coal tar oils, anthracene oil, etc. and pitches including special coal tar distillate fractions.

10 Certain aromatic derivatives including nitrobenzene, m-dinitrobenzene, o-nitrophenol, o-nitroanisole, o-nitroaniline, o- and m-nitrochlorobenzene, 2, 4, dinitrochlorobenzene, mono- and di-nitrotoluene, mono- and di-nitroxylenes, o-nitrodiphenyl,  $\alpha$ -nitronaphthalene and others, are also of great utility for special purposes either alone, in combination with one another, or when combined in varying percentages with aromatic or other hydrocarbon solvents.

15 Also useful in this process are high boiling petroleum fractions including lubricating fractions, cracked and straight run residues, asphalts, especially those melting below 220° F., furfural extracts of hydrocarbon oils including furfural extracts of lubricating fractions, and other solvent extracts which may be essentially aromatic or naphthenic in character.

20 These solvents are not exactly equivalent either 25 in their solvent power or in the utility for which the resulting coke solution may be employed. Each may have a special utility for different purposes. For example, a solution of raw petroleum coke in coal tar distillate may be of particular utility in the roofing industries and in the manufacture of synthetic boards, fiber boards and other slabs or forms. The solutions of raw coke in solvents such as cracked residues, heavy lubricating oils, and the like may be of particular utility as road oils and as a substitute for asphalt 30 in paints, tile, road surfacing, etc.

25 The solvents should in general have a melting and boiling point such that they remain liquid in the range of 300-600° F. and boil above about 500° F.

30 The coke may be taken into solution by 40 comminuting the raw coke, mixing it with the solvent, and heating the mixture with agitation to a suitable temperature until it becomes substantially uniform in character. Depending upon the volatile content of the coke, the temperature employed may vary substantially. With low volatile cokes comparatively higher temperatures and solvents of greater solvent power should be employed. With high volatile cokes lower temperatures and solvents with a lower solvent power 45 may be used.

50 The choice of the solvent will depend to some extent upon the amount of coke that is to be dissolved, and the properties of the finished article. In general solution temperatures of 300 to

650° F. may be employed. Coke may be comminuted to less than 100 mesh, if the higher temperatures are to be used, although larger particles can be dissolved where the volatile content and solvent power of the solvent permits use of lower temperatures.

In certain instances the coke may be entirely dissolved so far as can be ascertained. In other instances a large portion of the coke dissolves, generally a major portion, and leaves a minor proportion in the form of a stable suspension of minute particles apparently of microscopic size. These particles cannot be filtered out by ordinary methods, nor do they settle out upon long standing.

The solution thus produced may range from a material which is liquid at temperatures of 300 to 500° F. and which is a soft pitch at room temperatures, say 75 to 100° F., to a material which is hard and brittle at room temperature and may be a viscous paste at temperatures of 500° F. or higher.

The following examples are given to illustrate the invention but should not be construed as limiting it to the exact conditions or materials employed.

#### EXAMPLE I

A raw Mid-Continent petroleum coke was pulverized to pass a 48 mesh screen. The volatile content of the coke exclusive of water was 23.4%, this being capable of evolution only upon carbonization. The varying percentages of coke shown in Table I were mixed with a heavy coal tar oil at the temperatures indicated, mixing being carried out for a period of four to six hours. It will be observed that in proportions up to 50% of coke, uniform liquid solutions were obtained while at 71% of coke the material was liquid but contained minute particles of undissolved but highly dispersed material.

At room temperature the mixture containing 21% coke was a uniform glossy soft pitch useful in asphalt paints, as road oil or in the preparation of roofing materials such as shingles or as a roofing pitch. At 50% coke concentration a hard, ductile, glossy pitch was obtained useful as a substitute for high penetration roofing asphalt and in the preparation of tile and the like. At 71% concentration a very hard, brittle, uniform pitch was obtained which could be used as a binder for briquetting coal or coke, as a binder in the manufacture of carbon anodes and electrodes, or as a component of many building compositions in which a brittle hard asphalt is desirable.

Table I

| Mix No. | Formulation                |                            | Mixing Conditions |            | Softening Point (Ring and Ball) °F | Penetration 77°F/100g/5 sec. |
|---------|----------------------------|----------------------------|-------------------|------------|------------------------------------|------------------------------|
|         | Percent Raw Petroleum Coke | Percent Heavy Coal Tar Oil | Temp. °C          | Time Hours |                                    |                              |
| 1 1     | 21                         | 79                         | 350               | 4          |                                    |                              |
| 2 2     | 50                         | 50                         | 360               | 5          | 145                                | 12                           |
| 3 3     | 71                         | 29                         | 360               | 6          | 269                                | 0.1                          |

<sup>1</sup> Properties of product at mixing temperature—uniform liquid. Properties of product at room temperature—uniform glossy soft pitch.

<sup>2</sup> Properties of product at mixing temperature—uniform liquid. Properties of product at room temperature—uniform glossy medium hard ductile pitch.

<sup>3</sup> Properties of product at mixing temperature—liquid suspension. Properties of product at room temperature—very hard, brittle uniform pitch.

#### EXAMPLE II

A second series of samples were made with a raw petroleum coke from a Texas crude oil, and having 10.1% volatile content. It was pulverized to pass a 48 mesh screen. The percentages in the solutions and the conditions are shown in Table II.

Table II

| Mix No. | Formulation                |                            | Mixing Conditions |            | Softening Point (Ring and Ball) °F | Penetration 77°F/100g/5 sec. |
|---------|----------------------------|----------------------------|-------------------|------------|------------------------------------|------------------------------|
|         | Percent Raw Petroleum Coke | Percent Heavy Coal Tar Oil | Temp. °C          | Time Hours |                                    |                              |
| 4 1     | 21                         | 79                         | 350               | 6          |                                    |                              |
| 5 2     | 50                         | 50                         | 360               | 5          |                                    |                              |
| 6 3     | 71                         | 29                         | 340               | 5          | 134                                | 72                           |

<sup>1</sup> Properties of product at mixing temperature—liquid suspension with some undissolved coke.

<sup>2</sup> Properties of product at room temperature—dull soft pitch, grainy texture.

<sup>3</sup> Properties of product at mixing temperature—liquid suspension. No settling of undissolved coke.

<sup>4</sup> Properties of product at room temperature—dull rubbery compound. No separation of undissolved coke.

<sup>5</sup> Properties of product at mixing temperature—heavy viscous paste. Not uniform, does not liquefy.

<sup>6</sup> Properties of product at room temperature—solid, nonuniform lumps.

It will be observed that the products indicated in this example differ materially from those of Example I. The coke was dissolved to a substantially lesser extent. It is useful as a filled asphalt composition used for water proofing and sealing compounds. The sample containing the higher percentages of coke could be used as a paste or cement for filling cracks and the like. This example illustrates the effect of the decreased volatility on the type of product that can be produced.

It should be borne in mind that the coke used in these compositions must have a uniform volatility of not less than 8 to 10% throughout the coke to be treated. In certain coking operations a part of the coke is overheated locally and becomes hard, infusible and insoluble. The volatile content does not refer to an average volatility wherein lumps of such partially calcined coke of low volatility are contained, since such low volatile material can neither be dissolved nor dispersed. In selecting the coke care should be taken to eliminate such overheated portions.

#### EXAMPLE III

A raw petroleum coke of approximately 30% volatility, but nevertheless having no fusing point in that it would not deform with the application of mechanical pressure, was crushed to approximately 100 mesh and was mixed with equal portions by weight of a heavy cracked residuum of the fuel oil range. The mixture was heated at about 500° F. for five hours and was found to produce a uniform liquid mixture which set into a compound of the appearance and characteristics of asphalt at room temperature.

It is useful as a component of asphalt paints, in the preparation of road surfacing, roofing pitch and in the preparation of emulsions similar to asphalt emulsions.

It contained a small percentage of finely divided apparently solid particles which were nevertheless in stable suspension.

#### EXAMPLE IV

To the mixture of Example III was added about 5% of  $\alpha$ -nitronaphthalene at about 400° F. The

mixture thus produced was a uniform liquid, indicating that the solvent power of the fuel oil was increased by the addition of the aromatic derivative. Other aromatic compounds such as those hereinbefore listed behave similarly.

I claim as my invention:

1. A process which comprises mixing a raw, normally non-fusible coke produced by non-catalytic pyrolysis of highboiling liquid hydrocarbons, with an organic solvent therefor, said solvent being liquid in the range of 300-650° F. and boiling above 500° F., substantially completely dissolving said coke in said solvent at a temperature of 300-650° F., and recovering the substantially homogeneous solution thus formed, said coke having a volatile content of at least 8% which is capable of evolution only upon carbonization, the particles of said coke having the further property of being deformable under applied mechanical pressure when heated at about 500° F.

2. The process of claim 1 wherein the solvent is a petroleum hydrocarbon oil.

3. The process of claim 1 wherein the solvent is a coal tar distillate.

4. The process of claim 1 wherein the solvent is an aromatic hydrocarbon.

5. The process of claim 1 wherein the solvent is a nitro aromatic hydrocarbon.

6. The process of claim 1 wherein the solvent is a coal tar oil.

7. The process of claim 1 wherein the solvent is a hydrocarbon.

8. A pitch-like composition comprising a uniform solution of about 10-75% of raw petroleum coke having a volatile content of at least 8% which is capable of being removed only upon carbonization, and particles of which are capable

of being deformed upon application of mechanical pressure when heated to about 500° F., in an organic solvent liquid at 300-650° F. and boiling above 500° F.

5. The composition of claim 8 wherein the solvent is a petroleum hydrocarbon oil.

10. The composition of claim 8 wherein the solvent is a coal tar distillate.

11. The composition of claim 8 wherein the solvent is an aromatic hydrocarbon.

12. The composition of claim 8 wherein the solvent is a nitro aromatic hydrocarbon.

13. The composition of claim 8 wherein the solvent is a coal tar oil.

15. The composition of claim 8 wherein the solvent is a hydrocarbon.

HAROLD W. NELSON.

#### REFERENCES CITED

The following references are of record in the file of this patent:

#### UNITED STATES PATENTS

| Number    | Name           | Date          |
|-----------|----------------|---------------|
| 1,657,815 | Bates          | Jan. 31, 1928 |
| 1,702,899 | Howard         | Feb. 19, 1929 |
| 1,916,333 | Rose           | July 4, 1933  |
| 1,925,005 | Rose           | Aug. 29, 1933 |
| 2,037,147 | Radcliffe      | Apr. 14, 1936 |
| 2,194,574 | Snyder         | Mar. 26, 1940 |
| 2,301,322 | Reeves et al.  | Nov. 10, 1942 |
| 2,319,326 | Jenkner        | May 18, 1943  |
| 2,404,208 | Bangham et al. | July 16, 1946 |
| 2,453,641 | Reed           | Nov. 9, 1948  |

#### FOREIGN PATENTS

| Number  | Country       | Date         |
|---------|---------------|--------------|
| 316,897 | Great Britain | Aug. 6, 1929 |